

## UNITED STATES PATENT OFFICE.

WILLIAM MARSHALL, OF CHEADLE HULME, ENGLAND.

## MANUFACTURE OF FABRICS CONTAINING ARTIFICIAL SILK.

No Drawing.

Application filed October 13, 1923. Serial No. 668,419.

*To all whom it may concern:*

Be it known that I, WILLIAM MARSHALL, a subject of the King of Great Britain, residing in Cheadle Hulme, in the county of Chester and Kingdom of England, have invented certain new and useful Improvements in or Relating to the Manufacture of Fabrics Containing Artificial Silk, of which the following is a specification.

10 This invention relates to a process of manufacturing fabrics containing natural cellulose and artificial silk.

15 Piece goods containing artificial silk and having a mercerized finish have been made by weaving artificial silk with cotton which has been mercerized in the hank, because artificial silks such as viscose, "cuprammonium" silks, nitro-cellulose or the like are damaged by the ordinary mercerizing process.

20 According to the present invention, I make fabrics from unmercerized or incompletely mercerized yarn (hereinafter referred to as "incompletely mercerized yarn") and acetyl cellulose yarn and I then subject the fabric to the action of caustic alkali of mercerizing strength. The operation may be performed under tension in the usual mercerizing machines, or without tension when 30 a crêping effect is obtained.

25 I find that when strong caustic soda is used at a temperature of 15° C. or preferably lower, acetyl cellulose silk exhibits little or no contraction or loss of lustre and very little loss of weight. The effect of strong caustic soda is therefore strikingly different from that of the very dilute caustic soda which has been employed in conjunction with various salts for the purpose of 35 saponifying acetyl cellulose silk.

30 The dyeing properties of the acetyl cellulose silk do not appear to be materially affected except that the acetyl cellulose silk acquires more affinity for certain direct dyes. 40 The physical structure of the mercerized acetyl cellulose silk is somewhat altered and the irregular forms of the filament have largely disappeared and become more or less cylindrical. A pleasing lustre can be obtained by the treatment.

45 I may use caustic soda of specific gravity 1.24, but good results have also been obtained

50 at a specific gravity of 1.30. More dilute solutions may be used provided that they are capable of producing the mercerized effect on the natural cellulose fibre. I prefer to keep 55 the temperature as low as possible to protect the acetyl cellulose silk, since saponification is likely to occur at temperatures much above 15° C. Cooling may be effected by 60 the usual arrangements employed in connection with cloth mercerizing machines.

65 The mercerizing operation should be limited, i. e. the treatment should not be continued beyond the point at which the mercerizing effect is produced, because prolonged treatment may cause saponification of the acetyl cellulose silk.

70 The fabric is passed rapidly through the strong caustic soda by the continuous process, the pieces are squeezed through rollers, stretched as required and immediately washed in known manner. The caustic soda may be refrigerated.

75 After washing the goods are soured with cold dilute acid and washed again in cold water till neutral.

80 By this means, saponification is restricted so as to be substantially absent, i. e. less than one per cent, an amount which is without material influence on the properties of the acetyl cellulose yarn.

85 The goods may then be treated in the usual way for bleaching, dyeing, and finishing either in self colour or in a plurality of colours with or without shot effects.

90 The piece goods may contain dyed yarn (either acetyl cellulose or natural cellulose) in warp or weft or in both; in this case the yarn should be dyed with a fast dye.

95 To produce a crêping effect, the goods which may be specially woven for that purpose, if desired, are washed, soured and again washed without any tension either on the warp or weft.

I declare that what I claim is:—

1. The process of manufacturing fabrics of mixed artificial silk and mercerized cotton, which comprises weaving the fabric from incompletely mercerized cotton yarn, 100 and acetyl cellulose yarn, and then subjecting the fabric to the action of a caustic alkali mercerizing agent, wherein the action of such agent upon the acetyl cellulose is

substantially prevented by maintaining the caustic alkali at mercerizing strength at low temperatures.

2. Fabrics of cotton and acetyl cellulose silk which have been treated with caustic soda of about 1.24 to 1.30 specific gravity at a temperature not higher than about 15° C.

In witness whereof, I have hereunto signed my name this 2nd day of October, 1923, in the presence of two subscribing witnesses.

WILLIAM MARSHALL.

Witnesses:

JAMES HERBERT BRYDON,  
JOSEPH CHEETHAM.